

## UNITED STATES PATENT OFFICE

2,158,096

## LUBRICANT

James H. Werntz, Wilmington, Del., assignor to  
 E. I. du Pont de Nemours & Company, Wil-  
 mington, Del., a corporation of Delaware

No Drawing. Application April 24, 1936,  
 Serial No. 76,201

15 Claims. (CL 87—9)

This invention relates to lubricants and particularly to lubricants providing thin film lubrication.

The advantages of a high pressure lubricant become apparent when the present trend in design of automotive and other machine parts, and the increased strength of metal parts, due to the use of alloy steels, is considered. The pressures ordinarily found in well lubricated journal bearings do not exceed 2,000 lbs./sq. in. and, for conditions such as this, a film of heavy oil can be expected to remain between the rubbing surfaces. When gears are considered, where the contact between surfaces is of very small width, the bearing pressures often reach values as high as 25,000 lbs./sq. in. Under such extreme pressure, it is unlikely that any oil or grease can be obtained which will be viscous enough to prevent metallic contact. The result of the lack of a lubricating film between the rubbing surfaces results in scoring and scuffing of the gears.

Failure to maintain lubricant films on idle bearing surfaces is now well recognized as the cause of 70% to 80% of the wear occurring on cylinder walls of automotive and other internal combustion engines. When an engine is stopped, the oil film on the vertical surfaces soon drains off and, when the machine is again started up, an appreciable time elapses before the circulation provides oil for the formation of new lubricant films. An assistant which, when added to the motor oil, will prevent the separation of the oil film from the metal should prevent a large part of the wear now occurring.

Prior to this invention various assistants have been added to oils to improve their lubricating properties. Among such assisting materials which have been used are sulfur, sulfur chloride, sulfurized oil or oil containing naturally occurring sulfur, various heavy metal soaps and aluminum soaps, castor oil and, recently, aliphatic and aromatic halides. While some of these assistants, such as the sulfur and the organic halides improve the lubricating properties of the oil to a great extent, they have not proved to be satisfactory for use for the reason that they are corrosive or give rise to corrosive agents by hydrolysis or oxidation. Also, this corrosive action is greatly intensified by the presence of small amounts of water. Some of the alkyl halides are volatile and, hence, are soon lost. Other assistants such as the alkali and heavy metal soaps have proved to be of little value in improving the lubricating properties of the oils.

An object of this invention is to provide ma-

terials, which, when brought into contact with metal bearing surfaces, will form a lubricating film between such bearing surfaces, which lubricating film will adhere to the metal surfaces and resist high pressures. A further object of this invention is to provide materials which, when added to lubricating media, improve their properties, particularly their adhesiveness and resistance to high pressure. A still further object is to provide a method for retarding the wear, 10 scuffing and seizing of bearing surfaces, adapted to operate at high bearing pressures, by contacting such surfaces with materials which will form adherent films on such bearing surfaces, which films will not break down under high bearing 15 pressures. Other objects are to provide new compositions of matter and to advance the art. Still other objects will appear hereinafter.

These objects may be accomplished in accordance with my invention which comprises maintaining between relatively moving metallic bearing surfaces a film of a lubricating medium and at the same time chemically acting upon such surfaces by means of aliphatic acid esters of dibasic organic acids in which the aliphatic radical 25 contains at least 6 carbon atoms or their amine salts. When such lubricants are brought into contact with metal bearing surfaces, the esters appear to react chemically with the metal thereof to form a non-corrosive lubricating film which 30 will retard the wear of the bearing surfaces, will withstand high bearing pressures and will prevent metallic contact of the bearing surfaces under high bearing pressures. The films have exceptional lubricating properties at all pressures but 35 are particularly valuable at high bearing pressures and at high rubbing speeds. Such films will not be washed from the bearing surfaces by water, oil or organic solvents such as gasoline, naphtha and the like.

Preferably, the lubricating medium will be a hydrocarbon oil or grease. However, other oils or greases such as the animal and vegetable fats and oils may be employed. Also, preferably the esters of my invention will consist of the elements carbon, hydrogen and oxygen.

I preferably employ the esters of the dibasic acids in which the carboxyl groups are separated by at least two intervening carbon atoms. Among the compounds which I have found to be particularly effective for my purpose are the acid esters of citric, maleic, succinic and phthalic acids. Representative compounds are:

Octyl acid phthalate; cetyl acid phthalate; cetyl acid citrate; 9,10-octadecenyl acid citrate; 55

dodecyl acid succinate; dodecyl acid maleate; dodecyl acid phthalate; "Lorol" acid maleate (1); octyl acid phthalate; acid phthalate of the alcohols from petroleum; "Lorol" acid phthalate (1) and naphthenyl acid phthalate (2).

(1) The alcohol used in making these esters was a technical mixture of aliphatic primary monohydric alcohols containing from 8 to 14 carbon atoms obtainable by fractionally distilling the mixture of alcohols resulting from the carboxylic reduction of coconut oil and comprised approximately 12 parts of 8 carbon alcohol, 8 parts of 10 carbon alcohol, 57 parts of 12 carbon alcohol and 22 parts 14 carbon alcohol. This mixture is known to the trade as "Lorol" alcohol.

(2) This is a mixture of esters prepared from the mixture of alcohols obtained by the carboxylic reduction of a mixture of naphthenic acids from petroleum.

20 The term "bearing surfaces" as employed herein and in the claims will be understood to mean surfaces which mutually carry a load and move relatively to each other.

25 The addition of as small an amount as 0.05% of ester to an oil will have a noticeable effect. However, for practical purposes, it will generally be found desirable to use from about 0.5 to about

about 125 lbs. The machine provides for beam loadings up to 20 weights which corresponds to a pressure of 20,000 lbs./sq. in. on the full projected area of the drill rod. The bearing surface of the bushing is cut to a diameter 0.007 inch larger than the drill rod so that, before any wear occurs, the actual bearing surface is a line. As wear occurs, the bearing surface widens but seldom covers the bushing. After a test, the width of the bearing scar can be measured and an approximate value for the actual bearing pressure obtained. The values given in the following table represent the calculated actual bearing pressures which were reached in the test without failure of the film. These values represent film strength or 10 film resistance.

10 When subjected to the above test, a good grade of paraffin oil will withstand a pressure of only 3,000 to 6,000 lbs./sq. in. When an oil containing 20 sulfur is tested by the same method, such oil will show a film strength of about 20,000 lbs./sq. in. and will give a torque reading of over 4.0 lbs. ft. at this load.

20 In order to more clearly illustrate my invention and the advantageous results to be obtained 25 thereby the results of tests are given in the following table.

| 30 | No. | Compound                                  | Wt. percent | Oil medium | Allmen test results                     |                               | 30 |
|----|-----|-------------------------------------------|-------------|------------|-----------------------------------------|-------------------------------|----|
|    |     |                                           |             |            | Film strength 10000/lb/in. <sup>2</sup> | Friction at max. load lb. ft. |    |
| 35 | 1.  | None                                      |             | SAE. 30    | 6                                       | 0.6                           |    |
|    | 2.  | Octyl acid phthalate                      | 2           | do         | 74                                      | 2.2                           | 35 |
|    | 3.  | Cetyl acid phthalate                      | 2           | do         | 15                                      | 1.0                           |    |
|    | 4.  | Cetyl acid citrate                        | 2           | do         | 31                                      | 1.8                           |    |
|    | 5.  | 9,10-octadecenyl acid citrate             | 2           | do         | 13                                      | 1.4                           |    |
|    | 6.  | Dodecyl acid succinate                    | 2           | do         | 42                                      | 1.7                           |    |
|    | 7.  | Dodecyl acid maleate                      | 1           | do         | 38                                      | 1.8                           |    |
|    | 8.  | Dodecyl acid phthalate                    | 1           | do         | 42                                      | 1.4                           |    |
|    | 9.  | "Lorol" acid maleate                      | 1           | do         | 48                                      | 2.1                           |    |
|    | 10. | Octyl acid phthalate                      | 1           | Castor oil | 34                                      | 2.0                           | 40 |
|    | 11. | Acid phthalate of alcohols from petroleum | 2           | SAE. 30    | 33                                      | 2.5                           |    |
|    | 12. | "Lorol" acid phthalate                    | 2           | do         | 18                                      | 1.3                           |    |
|    |     | Naphthenyl acid phthalate                 | 2           | do         | 24                                      | 2.3                           |    |

45 1 The oil medium used in the above mixtures was an essentially naphthenic lubricating oil of characteristics corresponding to SAE. 30.

10% of the ester based on the oil. The actual concentration will depend on the particular compound or mixture of compounds employed and 50 the purpose to which the oil is to be put. For example, it is generally advisable to use higher concentrations of assistant in gear oils than would be employed in lubrication of internal combustion engines. Concentrations up to 20% 55 might be advantageously employed in special cases. Further, the amount added to the oil or other lubricating medium will be largely dependent upon the machinery in which it is applied and the area of the metal surfaces with which 60 it will be brought into contact.

The method of testing my compounds was that devised by J. O. Allmen (Oil and Gas Journal, 30, 109, 1931). This method consists of running a  $\frac{1}{4}$ " diameter drill rod between two halves of a 65 split bushing which is maintained stationary. The load on the bushing is controllable and provision is made for measuring the torque developed by the friction of the lubricant film. A hydraulic system for increasing the loading on the bushing until the oil film breaks and the metal seizes is provided. The rubbing speed is about 50 feet per minute and the method of loading is gradual, one weight being added to the loading lever each ten seconds. Each weight added to the loading 70 lever increases the pressure on the bushing by

The above tests merely illustrate the results obtained with a few of the compounds of my invention. Other compounds coming within my invention may be prepared from other aliphatic alcohols of 6 or more carbon atoms such as hexyl, cyclo-hexyl, decyl, hexadecyl, myricyl, tetradecyl, dodecyl, octa-decyl, linoleyl and like long chain alcohols or mixtures of two or more of them or the primary alcohols obtained by the oxidation 50 of petroleum or alcohols obtained by the reduction of the acids obtained from the petroleum or from the oxidation of petroleum. Likewise the higher primary alcohols of 6 or more carbon atoms obtained by the hydrogenation of carbon 55 atoms in the synthesis of methanol may be employed to prepare the esters of my invention. Also, one may employ esters of other acids such as: Mono-methyl succinic; dimethyl succinic; tri-methyl succinic; phenyl succinic; phenyl maleic; glutaric; adipic; suberic; fumaric; citraconic; citra-malic; iso-phthalic; tere-phthalic; hydro-phthalic; o-carboxy cinamic; o-carboxy hydrocinnamic; uvitic; iso-uvitic; naphthalic 65 diphenic and their homologues and isomers. 70

In accordance with my invention a single ester or a mixture of two or more of them may be employed. Generally, for reasons of better solubility or economy, mixtures of these materials will be employed. In preparing such mixture of 75

esters, mixtures of alcohols may be reacted with an acid, as in the "Lorol" acid maleate, "Lorol" acid phthalate and naphthenyl acid phthalate. The esters of my invention may be employed as the free acids or as the amine or ammonium salts.

The compounding of my esters with the oil can be accomplished by any one of a number of methods at present being employed in the petroleum industry for adding materials to the oils and greases. For example the oil can be heated until fluid enough to permit easy stirring when the assistant may be added. Agitation is then continued until the assistant has dissolved at which time the mixture may be cooled.

The compounds of my invention, when brought into contact with the metallic bearing surfaces, apparently react chemically therewith to form a film which is firmly adherent to the metal and at the same time presents a surface to the main body of oil with which the oil is compatible. This results in the formation of a mechanically resistant surface on the bearing and at the same time provides a bonding layer between the bearing and the oil, causing the oil and grease to adhere more firmly to the bearing surfaces. This is a particularly desirable and advantageous characteristic of my compounds particularly adapting them for use where the bearing surfaces are vertical and an ordinary oil tends to drain therefrom, as in the cylinders of internal combustion engines. My compounds do not induce rusting and cause little or no corrosion on most metals when admixed with oils in contact with such metals.

The fact that my compounds retain their extreme pressure lubricating characteristics in liquids other than oils and greases renders them particularly adapted for use as cutting oils, particularly in water emulsion. My compounds may be employed in other liquids than those mentioned in the examples. For instance, they may be employed in benzene, gasoline, diphenyl, diphenyl oxide and any other liquid which is non-corrosive to metal and in which the compounds may be dissolved, dispersed or emulsified.

The use of cutting oils in machining operations is well known. The cutting fluid has two functions; the first to provide a lubricant to reduce the friction between the cutting tool and the work, and the second to provide a means for cooling the work.

The general practice is to use either an oil or a dispersion of oil in water. The oils used vary considerably depending on the particular operation and may vary from a light mineral oil to a heavy mixture of mineral and animal oils. The water suspensions are usually made up from oils by the addition of dispersing agents of the Turkey red oil type. Recently the practice of adding sulfur or sulfur compounds has become common.

Die shaping of sheet metals and drawing of sheets, wires and tubes has also recently been improved by the use of a lubricant between the contacting surfaces.

Cutting oils are now generally made up by compounding about 30 parts of lard oil, one to five parts of sulfur, two to ten parts of a petroleum sulfonate or Turkey red oil and about 60 parts of mineral oil. This mixture is then used undiluted or dispersed in water which improves its cooling properties.

The lard oil, of course, breaks down under the high temperature conditions of use resulting in

the formation of disagreeably odorous materials. The presence of sulfur, as in motor and gear lubricants, is a possible source of corrosive material necessitating the careful washing of machined parts before use. These oils have also given considerable trouble from infection of the workmen which is only partially eliminated by the incorporation of a bactericide in the oil.

Wire drawing also requires an extreme pressure lubricant. Several types are in use but essentially they are the same as the ordinary cutting oils.

The pressures between the rubbing surfaces during all machining operations are obviously very high as they result in deformation of the metal. This is, therefore, another problem of extreme pressure lubrication.

My compounds may be used in water, oil or other suitable media as cutting oil compositions with the attending elimination of the odors and corrosiveness which are objectionable properties of most prior cutting oils. They will be effective at very low concentrations in oil and can be used in water directly without the use of an oil medium.

Other improvements similar to those observed on bearing lubrication should also result from such use. Decreased friction, safety from corrosion, and improved quality of the work are important results of their use.

The compounds of my invention are in general well known and the methods for making them are also well known and described in the literature. Accordingly, a detailed description of the methods to be employed for making the compounds referred to in this application is believed to be unnecessary.

While I have disclosed specific embodiments of my invention, it will be readily apparent to those skilled in the art that many modifications and variations may be made therein without departing from the spirit of my invention. Accordingly, the scope of my invention is to be limited solely by the appended claims construed as broadly as is permissible in view of the prior art.

I claim:

1. A high pressure lubricant comprising a lubricating oil or grease containing a small amount of an aliphatic acid-ester of a dibasic organic acid, the aliphatic radical containing at least 3 carbon atoms.

2. A high pressure lubricant comprising a lubricating oil or grease containing a small amount of an alkyl acid-ester of a dibasic organic acid in which the carboxyl groups are separated by at least 2 intervening carbon atoms, the alkyl radical containing at least 6 carbon atoms.

3. A high pressure lubricant comprising a lubricating oil or grease containing a small amount of an aliphatic acid-ester of a dibasic organic acid in which the carboxyl groups are separated by at least 2 intervening carbon atoms, the aliphatic radical containing at least 6 carbon atoms, said ester consisting of the elements carbon, hydrogen and oxygen.

4. A high pressure lubricant comprising a hydrocarbon lubricating oil or grease containing a small amount of an aliphatic acid-ester of a dibasic organic acid in which the carboxyl groups are separated by at least 2 intervening carbon atoms, the aliphatic radical containing at least 6 carbon atoms.

5. A high pressure lubricant comprising a hydrocarbon lubricating oil or grease containing a small amount of an alkyl acid-ester of a di-

basic organic acid in which the carboxyl groups are separated by at least 2 intervening carbon atoms, the alkyl radical containing at least 6 carbon atoms.

6. A high pressure lubricant comprising a hydrocarbon lubricating oil or grease containing a small amount of an aliphatic acid-ester of a di-basic organic acid in which the carboxyl groups are separated by at least 2 intervening carbon atoms, the aliphatic radical containing at least 6 carbon atoms, said ester consisting of the elements carbon, hydrogen and oxygen.

7. A lubricant for internal combustion engines consisting of a lubricating oil and a small amount of an acid-ester derived from an organic acid containing at least 2 carboxyl groups separated by at least 2 intervening carbon atoms and an aliphatic alcohol containing at least 6 carbon atoms.

8. A high pressure lubricant comprising a lubricating oil or grease containing a small amount of an alkyl acid-ester of phthalic acid, the alkyl radical containing at least 6 carbon atoms.

9. A high pressure lubricant comprising a lubricating oil or grease containing a small amount of octyl acid phthalate.

10. A high pressure lubricant comprising a lubricating oil or grease containing a small amount of naphthyl acid phthalate.

11. A high pressure lubricant comprising a lubricating oil or grease containing a small amount of an alkyl acid-ester of maleic acid, the alkyl radical containing at least 6 carbon atoms.

12. A high pressure lubricant comprising a lubricating oil or grease containing a small amount of "Lorol" acid maleate.

13. A lubricant for internal combustion engines consisting of a lubricating oil and a small amount of octyl acid phthalate.

14. A lubricant for internal combustion engines consisting of a lubricating oil and a small amount of naphthyl acid phthalate.

15. A lubricant for internal combustion engines consisting of a lubricating oil and a small amount of "Lorol" acid maleate.

JAMES H. WERNITZ.